

# UNITED STATES PATENT OFFICE.

WILLIAM CHARLES WAIN, OF NORTH SYDNEY, NEW SOUTH WALES, AUSTRALIA.

## CHLORATE EXPLOSIVE OF THE SPRENGEL CLASS.

1,240,272.

Specification of Letters Patent. Patented Sept. 18, 1917.

No Drawing.

Application filed March 19, 1915. Serial No. 15,582.

To all whom it may concern:

Be it known that I, WILLIAM CHARLES WAIN, a subject of the King of Great Britain and Ireland, residing at 63 Bellevue street, North Sydney, in the State of New South Wales, Commonwealth of Australia, have invented certain new and useful Improvements Relating to the Manufacture of Chlorate Explosives of the Sprengel Class, of which the following is a specification.

This invention relates to that class of explosives in which a cartridge of chlorate of potassium ( $KClO_3$ ) is immersed in and saturated by a suitable fluid, the resulting compound being capable of rapid combustion by detonation, though the solid and liquid elements are themselves inexplodable separately.

The object of this invention is to provide an improved saturating fluid which may be simply and economically compounded and from which free mineral acid is entirely absent, safety in storage being thereby insured without the necessity of alkaline washing; while the saturation of a cartridge of  $KClO_3$  with said fluid produces a compound of great explosive force.

The saturating fluid forming the subject of this invention is compounded of castor oil, raw linseed oil, petroleum (or its derivative kerosene), crude or refined, and fuming nitric acid sp. g. 1.5 ( $HNO_3$ ).

In compounding the fluid I take twenty (20) parts by measure of castor oil, twenty (20) parts of raw linseed oil, and three hundred and twenty (320) parts of petroleum (preferably but not necessarily refined). The castor oil and linseed oil are stirred into and dissolved by the petroleum, and a  $HNO_3$  is then added to the solution in a manner insuring even distribution, which effects nitration of the dissolved organic oils, and a viscous precipitate results. On standing the said precipitate is gradually and almost totally re-absorbed in the petroleum, a slight dark colored deposit which is valueless in this process adhering to the vessel. The solution is then decanted or poured off and is ready for the saturation of the chlorate cartridge.

In compounding this fluid as before stated it is essential that the quantity of  $HNO_3$  shall be sufficient and no more than sufficient,

to effectively nitrate the organic oils, so that no excess of acid is introduced to remain as free acid, and I have found that ten (10) parts of  $HNO_3$  added to the before-stated respective quantities of castor oil, linseed oil, and petroleum, will effect the required result.

The re-absorption by the petroleum of the viscous precipitate may be visually detected, but I have found that twenty four (24) hours is usually required for this purpose.

The fluid formed as the final product of the above described process has a specific gravity of approximately .816, is transparent and of a brown color; its rate of diffusion approximates to that of petroleum (re-absorbed) and is double that of nitro-benzol.

The saturation of the cartridge of  $KClO_3$  by the fluid produced as hereinbefore described, is effected in known manner and the combustion of the product is brought about by means of a detonator applied in accordance with the general practice in this class of explosives.

What I claim as my invention is:—

1. A saturating fluid for chlorate explosives of the Sprengel class, said fluid being a brown transparent liquid having a specific gravity of approximately .816 and a rate of diffusion of approximately double that of nitro-benzol, said fluid being formed by dissolving castor oil and raw linseed oil in petroleum and treating the said solution with fuming nitric acid.

2. A saturating fluid for chlorate explosives of the Sprengel class, said fluid being a brown transparent liquid having a specific gravity of approximately .816 and a rate of diffusion of approximately double that of nitro-benzol, said fluid being formed by treating equal parts of castor oil and raw linseed oil with sufficient petroleum to dissolve the said organic oils, and treating the said solution with sufficient nitric acid specific gravity 1.5 to completely nitrate said organic oils.

3. A saturating fluid for chlorate explosives of the Sprengel class, said fluid being a brown transparent liquid having a specific gravity of approximately .816 and a rate of diffusion of approximately double that of nitro-benzol, said fluid being formed by compounding castor oil, raw linseed oil, pe-

roleum and fuming nitric acid specific gravity 1.5 in or about the following proportions:—

5 Castor oil----- 20 parts by measure,  
Linseed oil----- 20 parts by measure,  
Petroleum ----- 320 parts by measure,  
Nitric acid----- 10 parts by measure.

4. A saturating fluid for chlorate explosives of the Sprengel class, said fluid being a brown transparent liquid having a specific gravity of approximately .816 and a rate of diffusion of approximately double that of nitro-benzol said fluid being formed by 10 treating equal parts of castor oil and raw linseed oil with sufficient petroleum to dissolve the said organic oils, and treating the 15 said solution with sufficient nitric acid, and

no more than sufficient acid, to completely nitrate the organic oils so that no excess is introduced to remain as free acid. 20

5. A process of manufacturing a saturating fluid for explosives of the Sprengel class, consisting of dissolving in petroleum equal parts of castor oil and raw linseed oil, nitrating the said organic oils by fuming nitric acid sp. g. 1.5 added to the solution, and allowing the resultant precipitate to be thrown down and subsequently re-absorbed by the petroleum, as herein described. 25

Signed at Sydney, New South Wales, Australia, this first day of February, 1915.

WILLIAM CHARLES WAIN.

Witnesses:

CHAS. HATTON,  
WM. NEWTON.